

Aug. 25, 1925.

1,551,197

A. S. KREBS

METHOD FOR CALCINING CRUDE LITHOPONE

Filed April 14, 1923

Fig. 1.



Fig. 2.



Inventor  
A. Sonnин Krebs.

by Francis J. Charles  
his Attorney.

## UNITED STATES PATENT OFFICE.

AUGUST SONNIN KREBS, OF WILMINGTON, DELAWARE, ASSIGNOR TO KREBS PIGMENT & CHEMICAL COMPANY, OF NEWPORT, DELAWARE, A CORPORATION OF DELAWARE.

## METHOD FOR CALCINING CRUDE LITHOPONE.

Application filed April 14, 1923. Serial No. 632,045.

To all whom it may concern:

Be it known that I, AUGUST SONNIN KREBS, a citizen of the United States of America, and resident of Wilmington, county of Newcastle, State of Delaware, have invented a certain new and useful Improvement in Methods for Calcining Crude Lithopone, of which the following is a true and exact description, reference 10 being had to the accompanying drawing, which forms a part thereof.

This invention relates to processes of manufacturing lithopone; and it has to do more particularly, though not in all respects 15 exclusively, with the calcination of crude lithopone in a continuous rotary furnace, most desirably of the muffle type, wherein the conditions of calcination are so controlled and regulated as to insure the production of high grade lithopone in a simpler, 20 more dependable and more economical way than has been available heretofore.

In the manufacture of lithopone, purified liquors or solutions of barium sulphide and 25 zinc sulphate are brought together in the precipitating or strike vats in the proper proportion and under proper conditions to produce a mixed precipitate of barium sulphate and zinc sulphide, which, after washing 30 and more or less complete drying, constitutes what is known as crude lithopone.

Long experience in the manufacture of lithopone by old methods and apparatus and protracted experiments and tests with new 35 methods and apparatus has demonstrated that a uniformly excellent product depends very largely on the conditions existing during the calcination of the crude lithopone which must be such that the mass under 40 treatment in all its parts is uniformly heated and maintained at the necessary or desirable calcining temperature for a necessary period and these conditions have been found to require that the mass while being 45 raised to and maintained at the necessary temperature should be constantly tumbled and mixed so that no portion remains in constant contact with or fixed relation to the walls of the furnace chamber and all 50 portions are exposed to the same heating conditions. It has also been found that for uniform good results it is highly desirable that the mass under treatment should for

the most part be held out of contact with the furnace walls and for this and other 55 reasons be maintained in a comparatively thick bed or layer in the furnace and for this and other reasons it has been found advisable to maintain in the rotating approximately horizontal muffle, which it is 60 preferred to use, a charge approximately half the cubic capacity of the muffle. In a rotating muffle through which the lithopone is fed this condition is conveniently maintained by providing the muffle with 65 a centrally located outlet orifice of small diameter at its outer end. A further object of my invention is to prevent the adherence of particles of lithopone to the walls of the muffle furnace. Even where the 70 muffle consists of a metal tube with smooth or unpolished inner walls there is a tendency for particles of lithopone to adhere to the wall, and consequently not mix with the bulk of the tumbling charge, consequently 75 such particles become overburned and moreover such adhering particles tend to promote the adherence of other particles and cause the formation of overburned crusts. It has been found that the adherence of 80 lithopone particles to the furnace wall can be prevented by causing vibrations to occur in the walls of the metal muffle at comparatively short intervals; such vibrations shake loose the adhering particles and insure that all parts of the charge shall be 85 calcined under similar and the best conditions.

Another object of the invention is to provide a method of calcining lithopone in 90 which the lithopone after having been raised to the necessary or desirable temperature is permitted to soak in its own heat for a period before its discharge from the muffle, the lithopone being tumbled during this 95 soaking period as it is during the heating up period.

Still another object of the invention is to provide for the cooling of the calcined lithopone before it is discharged from the muffle 100 or an extension of the muffle, so as to lessen the tendency to form zinc oxide on the exposure of the hot lithopone to the air.

The nature of the invention both as a new method and as to apparatus designed for the 105 practice of the method invention will be best

understood as described in connection with the drawing in which—

Figure 1 is a longitudinal sectional elevation of the improved furnace and

5 Figure 2, a cross section on line 2—2 of Fig. 1, illustrating a convenient device for periodically rapping the metallic muffle to cause vibration in its walls.

A is the heating furnace, B an oil jet. C, 10 C, walls supporting rollers C' which in turn support the tubular muffle D, through the metallic ring or tires E, E. F is an extension of the muffle C lying outside of furnace A, and having a heat insulating jacket F'.

15 G is a delivery orifice centrally located in the end of the muffle tube and of small diameter. H is a hopper having a tubular delivery spout H' in which works a conveyor I, the shaft I' of which has a sprocket wheel 70

20 I<sup>2</sup> secured to it. J is a sprocket wheel secured to the muffle D. K is a driving shaft having sprockets K' and K<sup>2</sup> which, through chains L and L', drive sprockets I' and J. M is a lever pivoted on shaft K carrying on 75

25 its free end a weighted roller M' which registers with the lifting cams N secured to the muffle, as shown in Fig. 2.

O is an air cooled muffle extension having 80 external ribs O' and a centrally located restricted discharge opening g. P is a belt conveyor for carrying away the calcined lithopone. Q and Q' are thermocouples. R indicates the level of the lithopone in the muffle. 85

35 In operation the crude lithopone is charged into the hopper H and fed from this hopper into the receiving end of the rotating muffle D by the action of the conveyor indicated at I. The construction at 90

40 at the receiving end of the muffle is such as to exclude air. The muffle D is kept in constant rotation by the described mechanism and may be slightly inclined toward its outer end to facilitate the travel of the lithopone through it. 95

45 As the lithopone travels through the muffle it is gradually raised to proper calcining temperature which it is preferred to maintain moderately low, say between 550° and 750° C., although it is 100

50 feasible to use somewhat lower temperatures and a temperature of as high as 900° C. or thereabouts may be employed under some circumstances. The time of 105

55 treatment will naturally vary with the temperature to which the lithopone is raised but within the range of temperatures preferred the period of calcination will be in the neighborhood of from fifty to twenty-five minutes. 110

60 The lithopone is maintained in the rotating muffle in a comparatively deep layer or bed approximating half the cubic capacity of the muffle and this is best accomplished by providing the delivery end of the muffle with a centrally located 115

65 delivery orifice of relatively small diameter, as indicated at G. The exact proportion and volume of the lithopone to the cubic capacity of the muffle is not at all important so long as a bed or layer of substantial thickness is maintained. 70

The lithopone under treatment is, in the apparatus shown, constantly stirred and tumbled by the rotation of the muffle and this tumbling action is of great importance in securing substantially uniformity of condition and exposure to heat of the whole mass of lithopone under treatment. 75

The tendency of particles of lithopone to adhere to the walls of the muffle and become overburned is overcome by causing frequent vibrations in the walls of the metallic muffle and a convenient device for striking frequent periodical blows causing such vibration is the weighted lever M which is raised by the cams N and periodically allowed to fall upon the muffle D. 80

I have, as already stated, discovered that material advantages are secured by permitting the lithopone after it is raised to the desired calcining temperature to soak in its own heat for a period before its final delivery out of the muffle. Such a heat soaking of the lithopone is provided for in the apparatus shown by the muffle attachment F having a heat insulating jacket F' which is attached to the muffle outside of the furnace A so that, after being raised to the proper temperature the lithopone in the extension F is permitted to soak in its own heat while being constantly agitated and tumbled as 90

it is in the muffle itself. 95

It is, I believe, advantageous in calcining lithopone in a muffle of whatever construction and mode of operation that the lithopone should be cooled to some material degree before it is exposed to the air and in effect before it escapes from the atmospheric conditions existing in the muffle. This I provide for by attaching to the end of the muffle a cooling extension indicated at O which, as 100

shown, is intended to be air cooled and provide ribs O' but which, of course, can be cooled in any convenient way. This extension, as shown, is secured to the end of the 105

extension F and rotates with the muffle and is provided with a centrally located delivery orifice g of small diameter so that the conditions as to tumbling and thickness of the 110

layer are maintained in this extension. In the construction shown the small delivery orifice G or g insures not only that a properly deep bed of lithopone should be maintained but also provides against the entrance of air at the delivery end of the muffle and its extensions, a constant outward current of 115

gas and vapors generated in the muffle passing through the small delivery orifices. 120

This apparatus described embodies also

newly invented features which are the subject matter of my application filed June 21, 1924, Serial Number 721,436.

Having now described my invention, what I claim as new and desire to secure by Letters Patent, is:

1. The method of calcining crude lithopone which consists in charging the crude lithopone into a substantially horizontal tubular rotating furnace maintained at calcining temperature, regulating the amount of the furnace charge so that it will not substantially exceed half the cubic capacity of the furnace, constantly stirring and turning the charge by the rotation of the furnace and maintaining a substantially non-oxidizing atmosphere in the furnace during the calcination of the charge.

2. The method of calcining crude lithopone which consists in charging the crude lithopone into a substantially horizontal tubular rotating furnace maintained at calcining temperature, regulating the amount of the furnace charge so that it will not substantially exceed half the cubic capacity of the furnace, constantly stirring and turning the charge by the rotation of the furnace, preventing adhesion of particles of the charge to the furnace walls by causing said walls to vibrate and maintaining a substantially non-oxidizing atmosphere in the furnace during the calcination of the charge.

3. The method of calcining crude lithopone which consists in charging the crude lithopone into a substantially horizontal tubular rotating furnace, maintaining a calcining temperature in said furnace by heat transmitted through the walls thereof, regulating the amount of the furnace charge so that it will not substantially exceed half the cubic capacity of the furnace, constantly stirring and tumbling the lithopone under treatment by the rotation of the furnace and maintaining a substantially non-oxidizing atmosphere in the furnace during the calcination of the charge.

4. The method of calcining crude lithopone which consists in continuously charging the crude lithopone into one end of a substantially horizontal tubular rotating furnace causing the lithopone to move continuously through the furnace to a discharge opening at its other end, regulating the feed of lithopone into and through the furnace so that it will not occupy substantially more than half of the cubic capacity of the furnace, maintaining a calcining temperature in said furnace by heat transmitted through the walls thereof, constantly stirring and tumbling the lithopone under treatment by the rotation of the furnace, preventing adhesion of particles of lithopone to the walls of the furnace by causing said walls to vibrate and maintaining a substan-

tially non-oxidizing atmosphere in the furnace during the calcination of the charge.

5. The method of calcining crude lithopone which consists in continuously charging crude lithopone into one end of a horizontal rotating tubular furnace, continuously feeding the lithopone through the furnace to a discharge opening at its other end, maintaining the lithopone in the furnace in a deep bed approximately but not materially exceeding half the cubic capacity of the furnace, maintaining the furnace at calcining temperature by heat transmitted through the walls of the furnace, maintaining a substantially non-oxidizing atmosphere in the furnace and continuously tumbling the deep charge in the furnace by the rotation of the furnace.

6. The method of calcining crude lithopone which consists in continuously charging crude lithopone into one end of a horizontal rotating tubular furnace, continuously feeding the lithopone through the furnace to a discharge opening at its other end, maintaining the lithopone in the furnace in a deep bed approximately but not materially exceeding half the cubic capacity of the furnace, maintaining the furnace at calcining temperature by heat transmitted through the walls of the furnace, maintaining a substantially non-oxidizing atmosphere in the furnace continuously tumbling the deep charge in the furnace by the rotation of the furnace and preventing the adherence of lithopone particles to the furnace walls by causing vibration of the furnace wall.

7. The method of calcining crude lithopone which consists in continuously charging crude lithopone into one end of a horizontal rotating tubular furnace in a stream of small section, maintaining the lithopone in the furnace in a layer approximately but not materially exceeding half the capacity of the furnace by causing it to discharge in a thin stream through a small centrally located opening at the discharge end of the furnace, heating the charge by heat transmitted through the wall of the furnace, maintaining a substantially non-oxidizing atmosphere in the furnace and continuously tumbling the furnace charge by the rotation of the furnace.

8. The method of calcining crude lithopone which consists in feeding it through a horizontal rotatable tubular furnace, maintaining the lithopone in a deep bed in the furnace, heating the charge by heat transmitted through the front portion of the walls of the furnace but not through the walls of the rear or delivery end thereof, permitting the calcined charge to soak in its own heat as it passes through the unheated end of the furnace, tumbling the

charge throughout the length of the furnace by rotating the furnace and maintaining a substantially non-oxidizing atmosphere throughout the furnace.

- 5 9. The method of calcining crude lithopone which consists in feeding it longitudinally through an externally heated muffle in a substantially non-oxidizing atmosphere and cooling the calcined product by passing
- 10 it through an externally cooled muffle extension in which the non-oxidizing atmosphere is also maintained.

10. The method of calcining crude lithopone which consists in feeding it longitudinally through an externally heated muffle permitting the calcined product to soak in its own heat as it passes through a rear non-externally heated section of the muffle in a substantially non-oxidizing atmosphere and

15 20 cooling the calcined product by passing it through an externally cooled muffle extension in which the non-oxidizing atmosphere is also maintained.

11. The method of calcining crude lithopone which consists in feeding it through a horizontal rotatable tubular furnace, maintaining the lithopone in a deep bed in the furnace, heating the charge by heat trans-

mitted through the front portion of the walls of the furnace but not through the walls of the rear or delivery end thereof, permitting the calcined charge to soak in its own heat as it passes through the unheated end of the furnace, cooling the calcined lithopone by passing it through an externally cooled furnace extension, tumbling the charge throughout the length of the furnace and its extension by rotating the furnace and maintaining a substantially non-oxidizing atmosphere throughout the furnace and

30 35 40 its extension.

12. The method of calcining crude lithopone which consists in passing it through a horizontal externally heated rotatable tubular furnace in a deep layer, heating the charge by heat transmitted through the walls of the furnace, continuously tumbling the charge in the furnace by the rotation of the furnace, cooling the calcined lithopone by passing it through an externally cooled furnace extension and maintaining a substantially non-oxidizing atmosphere in the furnace and its externally cooled extension.

45 50

A. SONNIN KREBS.